

3,397,096

**THICKENED INORGANIC OXIDIZER SALT EXPLOSIVE SLURRY SENSITIZED WITH A SOLUBLE POLYFLAVONOID**

Errol Linton Falconer, St. Hilaire, Quebec, and Cornelius James Noel Kelly, Beloeil, Quebec, Canada, assignors to Canadian Industries Limited, Montreal, Quebec, Canada  
No Drawing. Filed Nov. 20, 1967, Ser. No. 684,538  
Claims priority, application Canada, Dec. 6, 1966,  
977,354  
8 Claims. (Cl. 149—39)

**ABSTRACT OF THE DISCLOSURE**

The sensitivity of slurry explosive compositions comprising inorganic oxygen-supplying salts, a fuel, a thickener and a liquid carrier is substantially improved by incorporating in the composition a soluble polyflavonoid and a common solvent for the polyflavonoid and the inorganic salt.

This invention relates to explosive compositions comprising essentially an inorganic oxygen-supplying salt, a sensitizer, a fuel, a thickener and a mutual solvent for the inorganic salt and the sensitizer. In particular, the invention relates to a means whereby the sensitivity of such explosive compositions may be substantially improved.

Explosive compositions comprising an oxygen-supplying salt such as, for example, ammonium nitrate, and a sensitizer and/or fuel together with a fluid solvent, disperser or carrier such as water, are known. These compositions are commonly referred to as slurry explosive compositions or, more generally, as slurry explosives. Such slurry explosives may range in degree of firmness or consistency from highly viscous, plastic-like extrudable compositions to less viscous pumpable or pourable fluid-like mixtures.

Slurry explosive compositions of the aforementioned types normally contain as essential ingredients widely known sensitizing and power enhancing materials and fuels such as, for example, finely divided light metal, finely divided carbon and the like. In some cases, it is advantageous to add a self-explosive ingredient such as particulate TNT, PETN, or smokeless powder to further improve the sensitivity or strength or both of the slurry explosives and thereby insure detonation and propagation. A wide range of such compositions are now known to the art.

For optimum reliability the known sensitizers employed in slurry explosives are either self-explosives or relatively expensive materials such as very finely divided light metal powders. Without such sensitizers, these slurry explosive compositions tend to be detonable only in large diameter charges with large primers. It has thus been necessary for the manufacturer of explosives to employ relatively large quantities of sensitizing material and fuel in slurry explosives in order to insure detonation and propagation. Such compositions, as well as being relatively expensive, are hazardous to handle and require special and costly precautions in manufacture, transportation, storage and use. Slurry explosive compositions containing self-explosives are, in turn, in most jurisdictions subject to regulatory restrictions in transportation and storage. Those that contain reactive sensitizers such as, for example, paint-fine aluminium powder, tend to deteriorate and lose sensitivity on storage.

It has now been found that the aforementioned disadvantages may be overcome by employing as a sensitizer in slurry explosive compositions a soluble polyflavonoid.

It is, therefore, an object of the present invention to provide a means whereby the sensitivity of a slurry explosive composition may be increased.

Another object of the invention is to provide a slurry explosive composition which may be detonated in boreholes of small diameter.

Another object of the invention is to provide a sensitive slurry explosive composition which is devoid of any self-explosives or other hazardous material.

10 A further object of the invention is to replace the known reliable sensitizers in slurry explosive compositions with a sensitizer that is much less costly and easily available.

These and other objects of the invention will become 15 apparent from a consideration of the following description and claims.

The improved explosive composition of this invention comprises essentially at least one inorganic oxygen-supplying salt, at least one soluble polyflavonoid, a fuel, a 20 thickener and a mutual solvent, usually water, for the inorganic salt and the polyflavonoid.

The addition of a soluble polyflavonoid to a slurry explosive composition has the surprising and desirable effect of substantially increasing the sensitivity of the 25 composition.

It is thus now possible to prepare useful and powerful, slurry explosive compositions which, though devoid of any self-explosive ingredient, may be detonated with ease in boreholes of small diameters. It is similarly now 30 possible to prepare such compositions even containing additional sensitizing material such as, for example, finely divided aluminium, aluminium alloy, silicon, ferrosilicon or ferrophosphorus or self-explosives which are more reliable to detonation and propagation than heretofore 35 and which may be detonated in smaller diameter and with the use of smaller priming charges that has heretofore been possible.

Preferred blasting slurry explosive compositions of this 40 invention contain from 30 to 90% by weight of at least one inorganic oxygen-supplying salt, from 0.1 to 25% by weight of a soluble polyflavonoid, from 1 to 30% by weight of a mutual solvent for the inorganic salt and the polyflavonoid, from 0.1 to 10% by weight of thickener and from 0 to 40% by weight of fuel, the proportions of 45 the ingredients being such that the oxygen balance of the total composition is from +15 to -35 grams of oxygen per 100 grams of finished explosive.

A preferred inorganic oxygen-supplying salt for inclusion in the explosive compositions of this invention is 50 ammonium nitrate. It is in some cases advantageous to replace some, suitably up to 50% or even up to 90%, of the ammonium nitrate by other metal nitrates such as sodium, barium, potassium and calcium nitrates. The 55 particle size of the inorganic oxygen-supplying salts is not critical and powdered, granulated, or prilled forms may be used and part of the salts may be predissolved in all or part of the solvent.

A preferred mutual solvent for the oxidizing salt and the soluble polyflavonoid is water. However, quite large 60 proportions of the water may be replaced by organic solvents such as formamide, dimethyl sulfoxide and the lower glycols and alcohols. These solvents are polar liquids, readily miscible with water in all proportions and are effective solvents for ammonium nitrate 65 and other inorganic salts. The replacement of water is limited only by the lack of solubility of the polyflavonoid in solvent mixtures of low water content.

Where employed, the aluminium or aluminium alloy or other energetic metal or metalloids suitable for use in 70 the explosive composition of this invention must be in finely divided form and may most suitably range from a



effect of substantially increasing the sensitivity of the compositions. Slurry explosives of this type having an oxygen balance outside the range of +15 to -35 grams of oxygen per 100 grams of finished explosive make very uneconomical use of the available energy. It is preferred, therefore, that quantities of polyflavonoid sensitizer and fuel used be such that the oxygen balance of the composition is within the range +15 to -35.

It will be appreciated by those skilled in the art that the principal advantage to be enjoyed through the use of the polyflavonoid sensitized slurry explosive compositions of the invention lies in the utilization of non-self-explosive slurry composition. That is, slurry compositions comprising oxygen-supplying salts, a solvent for the oxygen-supplying salts and a fuel may now, by the addition of a suitable quantity of a polyflavonoid, be employed as practical and reliable commercial explosives possessing the additional advantages of low cost and great handling safety. Where it is desired to include in such compositions additional strength ingredients such as powdered light metal fuels or self-explosives, the use of the polyflavonoid sensitizers provides compositions which may be detonated in smaller diameter charges or with lower strength primers than has heretofore been possible.

The polyflavonoid sensitizers provide an additional function in controlling the density of the explosive compositions since they are effective agents in preventing or arresting the dissipation of minute bubbles of air which have been entrained or occluded in the slurry mixture. Such air bubbles are normally incorporated in slurry explosive compositions by the lifting and folding of the mixture which occurs during the mechanical mixing of the ingredients or, alternatively, air is entrapped into the mixture in the voids of the dry ingredients. Such control of density is useful in permitting different loading and cartridge densities.

What we claim is:

1. An explosive composition comprising essentially at least one inorganic oxygen-supplying salt, a soluble polyflavonoid, a mutual solvent for the inorganic oxygen-supplying salt and the soluble polyflavonoid, a thickener and a fuel, the proportions of the ingredients being such that the oxygen balance of the total composition is from about +15 to about -35 grams of oxygen per 100 grams of finished explosive.

2. An explosive composition as claimed in claim 1

wherein the fuel is selected from the group consisting of carbonaceous material, particulate organic explosives, particulate light metal or metalloids, sulphur, carbon, urea and mixtures thereof.

5 3. An explosive composition as claimed in claim 1 wherein the mutual solvent is water.

4. An explosive composition as claimed in claim 1 wherein the mutual solvent comprises a mixture of water and a miscible organic solvent selected from the group consisting of formamide, dimethyl sulfoxide, lower glycols and alcohols, the proportions being such as to permit a solubility of not less than 5 parts of polyflavonoid per 100 parts of the solvent mixture.

5 5. An explosive composition as claimed in claim 1 wherein the oxygen supplying salt is selected from the group consisting of the nitrates of ammonia, sodium, potassium, barium, calcium and mixtures thereof.

6. An explosive composition as claimed in claim 1 wherein the soluble polyflavonoid is present as its sodium salt.

7. An explosive composition as claimed in claim 2 wherein the particulate organic explosive is selected from the group consisting of trinitrotoluene, pentaerythritol tetranitrate, cyclotrimethylenetrinitramine, mixture of trinitrotoluene and cyclotrimethylenetrinitramine, mixture of pentaerythritol tetranitrate, smokeless powder, nitrocellulose, nitrostarch and mixtures thereof.

8. An explosive composition comprising essentially between about 30% and about 90% by weight of an inorganic oxygen-supplying salt, between about 0.1% and 25% by weight of a soluble polyflavonoid, from about 1% to about 30% by weight of a mutual solvent for the inorganic oxygen-supplying salt and the soluble polyflavonoid, from about 0.1% to about 10% by weight of a thickener and from 0 to 40% by weight of a fuel, the oxygen balance of the total composition being from about +15 to about -35 grams of oxygen per 100 grams of finished explosive.

40 **References Cited**  
UNITED STATES PATENTS

3,369,945 2/1968 Craig et al. ----- 149-44 X

BENJAMIN R. PADGETT, *Primary Examiner.*

45 S. J. LECHERT, JR., *Assistant Examiner.*